

[54] PROCESS FOR THE PRODUCTION OF A PRESSURE-SENSITIVE CARBONLESS COPY SHEET USING MICROCAPSULES FORMED IN SITU IN A RADIATION CURABLE BINDER

[75] Inventors: Yu-Sun Lee, Parma Heights; Dale Richard Shackle, Chillicothe, both of Ohio

[73] Assignee: The Mead Corporation, Dayton, Ohio

[21] Appl. No.: 800,561

[22] Filed: May 25, 1977

[51] Int. Cl.<sup>2</sup> ..... B05D 3/06

[52] U.S. Cl. ..... 428/307; 162/184; 282/27.5; 252/316; 427/54; 427/150; 427/152; 428/914

[58] Field of Search ..... 427/53, 54, 150, 151, 427/152; 428/307, 327, 914; 252/316; 162/184; 282/27.5

[56] References Cited

U.S. PATENT DOCUMENTS

|           |         |                 |       |         |
|-----------|---------|-----------------|-------|---------|
| 3,242,051 | 3/1966  | Hiestand et al. | ..... | 427/354 |
| 3,405,071 | 10/1968 | Reyes           | ..... | 252/316 |
| 3,432,327 | 3/1969  | Kan et al.      | ..... | 252/316 |
| 3,552,986 | 1/1971  | Bassemir et al. | ..... | 427/54  |

Primary Examiner—John H. Newsome

Attorney, Agent, or Firm—Steven H. Cogle; Wilson G. Palmer

[57] ABSTRACT

A process is provided for the production of a coating composition containing microcapsules having a hydrophilic core for use in the manufacture of pressure-sensi-

tive carbonless transfer papers comprising the following steps. A hydrophilic emulsion component is prepared by dispersing at least one chromogenic material being soluble in the hydrophilic liquid. A hydrophobic emulsion component is prepared by dispersing an emulsifier in a radiation curable hydrophobic liquid. A first wall-forming material and a second wall-forming material are added to the hydrophobic emulsion component, with mixing. The first and second wall-forming materials are soluble in the hydrophobic emulsion component, and the first wall-forming material is reactive with the second wall-forming material to form a polymeric capsule wall. The resultant polymeric capsule wall is substantially insoluble in the hydrophilic and the hydrophobic emulsion components. The hydrophobic emulsion component is mixed together with the hydrophilic emulsion component to form an emulsion containing droplets of the hydrophilic emulsion component dispersed in the hydrophobic emulsion component. Mixing is maintained for a period of time sufficient to allow the first and second wall-forming materials to react to form a dispersion of microcapsules in the hydrophobic emulsion component. The formed microcapsules have capsule walls substantially impermeable to the hydrophobic and the hydrophilic emulsion components.

Pressure-sensitive carbonless transfer paper may be produced by applying the dispersion of the microcapsules prepared as above to a substrate, and curing the dispersion by subjecting the dispersion on the substrate to radiation for a period of time sufficient to cure the radiation curable hydrophobic liquid, thereby producing a tack-free, resinous film on the substrate.

25 Claims, No Drawings

PROCESS FOR THE PRODUCTION OF A  
PRESSURE-SENSITIVE CARBONLESS COPY  
SHEET USING MICROCAPSULES FORMED IN  
SITU IN A RADIATION CURABLE BINDER

BACKGROUND OF THE INVENTION

1. Field of the Invention

This invention relates to the production of radiation curable microcapsular coating compositions. In particular, it relates to the production of microcapsules containing a hydrophilic core by reaction of two wall-forming materials in a hydrophobic liquid wherein the hydrophobic liquid is a radiation curable organic liquid. In one embodiment of this invention, the encapsulated hydrophilic liquid contains a chromogenic material soluble in the encapsulated hydrophilic liquid. A dispersion of these microcapsules can be coated on a substrate and cured by radiation to give a pressure-sensitive carbonless copy sheet having a transfer coating.

2. Prior Art

The production of microcapsules containing an encapsulated oily (hydrophobic) liquid wherein the microcapsule walls are produced by reaction of polyisocyanate and a second wall-forming material is described in U.S. Pat. No. 3,796,669 to Kiritani et al. Both the polyisocyanate wall-forming material and the second wall-forming material are mixed with the oily liquid. The mixed oily liquid is dispersed into an aqueous continuous phase to form a dispersion of oil drops and the temperature is raised to initiate the reaction on the surface of the oil drops thus encapsulating the oil drops with the reaction product of the polyisocyanate and second wall-forming material. A catalyst for the reaction may also be added to the oily liquid.

Carbonless copy paper, briefly stated, is a standard type of paper wherein during manufacture the backside of the paper substrate is coated with what is referred to as a CB or transfer coating, the CB coating containing one or more chromogenic materials, generally in capsular form. At the same time the front side of the paper substrate is coated during manufacture with what is referred to as a CF coating, which contains one or more chromogenic materials capable of producing a color with the encapsulated CB chromogenic material. Both the chromogenic materials remain in the coatings on the respective back and front surfaces of the paper in substantially colorless form. This is true until the CB and CF coatings are brought into overlying relationship and sufficient pressure, as by a typewriter, is applied to rupture the CB coating to release the encapsulated chromogenic material. At this time the chromogenic material contacts the CF coating and reacts with the chromogenic material therein to form a colored image. Carbonless copy paper has proved to be an exceptionally valuable image transfer media for a variety of reasons, only one of which is the fact that until a CB coating is placed next to a CF coating both the CB and CF coatings are in an inactive state as the coreactive elements are not in contact with one another until pressure is applied. Patents relating to carbonless copy paper products are:

- U.S. Pat. No. 2,712,507 (1955) to Green
- U.S. Pat. No. 2,730,456 (1956) to Green et al.
- U.S. Pat. No. 3,455,721 (1969) to Phillips et al.
- U.S. Pat. No. 3,466,184 (1969) to Bowler et al.
- U.S. Pat. No. 3,672,935 (1972) to Miller et al.

A disadvantage of coated paper products such as carbonless transfer paper stems from the necessity of applying a liquid coating composition containing the color forming ingredients during the manufacturing process. In the application of such coatings, volatile organic solvents are sometimes used which then in turn requires evaporation of excess solvent to dry the coating thus producing volatile solvent vapors. An alternate method of coating involves the application of the color forming ingredients in an aqueous slurry, again requiring removal of excess water by drying. Both methods suffer from serious disadvantages. In particular, the organic solvent coating method necessarily involves the production of generally volatile solvent vapors, creating both a health and a fire hazard in the surrounding environment. When using an aqueous solvent system the water must be evaporated which involves the expenditure of significant amounts of energy. Further, the necessity of a drying step requires the use of complex and expensive apparatus to continuously dry a substrate which has been coated with an aqueous coating compound. A separate but related problem involves the disposal of polluted water. The application of heat not only is expensive, making the total paper manufacturing operation less cost effective, but also is potentially damaging to the chromogenic materials which are generally coated onto the paper substrate during manufacture. High degrees of temperature in the drying step require specific formulation of coating compositions which permit the use of excess heat. The problems encountered in the actual coating step are generally attributable to the necessity for a heated drying step following the coating operation.

The novel process and liquid coating composition of this invention are superior to those used in the prior art microcapsular coating of substrates in that they do not need an organic solvent or water in their coating composition, thus avoiding the disadvantages associated with solvent removal during drying. The liquid radiation curable substance is a solvent for the wall-forming material in the hydrophobic liquid. The liquid radiation curable substance cures by radiation to give a tack-free film containing microcapsules. The cured film acts as a binder to adhere the microcapsules to the substrate.

In general, patents concerned with the production and application of liquid resin compositions containing no volatile solvent which are subsequently cured by radiation to a solid film are:

- U.S. Pat. No. 3,551,235 (1970) to Bassemir et al.
- U.S. Pat. No. 3,551,246 (1970) to Bassemir et al.
- U.S. Pat. No. 3,551,311 (1970) to Nass et al.
- U.S. Pat. No. 3,558,387 (1971) to Bassemir et al.
- U.S. Pat. No. 3,661,614 (1972) to Bassemir et al.
- U.S. Pat. No. 3,720,534 (1973) to Macaulay et al.
- U.S. Pat. No. 3,754,966 (1973) to Newman et al.
- U.S. Pat. No. 3,772,062 (1973) to Shur et al.
- U.S. Pat. No. 3,772,171 (1973) to Savageau et al.
- U.S. Pat. No. 3,801,329 (1974) to Sandner et al.
- U.S. Pat. No. 3,819,496 (1974) to Roskott et al.
- U.S. Pat. No. 3,847,768 (1974) to Kagiya et al.
- U.S. Pat. No. 3,847,769 (1974) to Garratt et al.

These compositions generally also contain a pigment or dye. Such resin compositions are useful for protective coatings and fast drying inks. U.S. Pat. No. 3,754,966 describes the production of an ink releasing dry transfer element which can be used as a carbon paper or typewriter ribbon. It is significant to note here that the particular radiation cured coating must be compatible with

the reaction of CB and CF chromogenic materials to form a color. Such color forming reactions are generally of a sensitive or delicate nature and are not generally compatible with the compositions found in the prior art.

The novel liquid coating compositions of this invention contain microcapsules having an aqueous core liquid. The microcapsule walls are produced by a reaction of two wall-forming materials in a radiation curable hydrophobic liquid. Prior to the discovery of this invention, it was not known that such microcapsules could be produced in situ in radiation curable liquid compositions. For purposes of this disclosure, a tack-free film is one which will separate cleanly from a cotton ball lightly pressed against the film. The cotton fibers will not adhere to the film surface.

An especially preferred application of the process of this invention is in the continuous production of a manifold carbonless form. The continuous production of a manifold paper product would require simultaneous coating, simultaneous drying, simultaneous printing, and simultaneous collating and finishing of a plurality of paper substrates. Thus, Busch in Canadian Pat. No. 945,443 indicates that in order to do so there would be a minimum wetting of the paper web by water during application of the CB emulsion coat. For that purpose a high solids content emulsion is used and special driers are described in Busch. However, because of the complexities of the drying step, this process has not been commercially possible to date. More particularly, the drying step involving solvent evaporation and/or water evaporation and the input of heat does not permit the simultaneous or continuous manufacture of manifold forms. In addition to the drying step which prevents continuous manifold form production the necessity for the application of heat for solvent evaporation is a serious disadvantage since aqueous coatings require that special grades of generally more expensive paper be employed and even these often result in buckling, distortion or warping of the paper by the water present in the coating. Additionally, aqueous coatings are generally not suitable for spot application or application to limited areas of one side of a sheet of paper. They are generally suitable only for application to the entire surface area of a sheet to produce a continuous coating.

Another problem which has been commonly encountered in attempts to continuously manufacture manifold forms has been the fact that a paper manufacturer must design paper from a strength and durability standpoint to be adequate for use in large variety of printing and finishing machines. This requires a paper manufacturer to evaluate the coating apparatus of the forms manufacturers he supplies in order that the paper can be designed to accommodate the apparatus and process designed exhibiting the most demanding conditions. Because of this, a higher long wood fiber to short wood fiber ratio must be used by the paper manufacturer than is necessary for most coating, printing or finishing machines in order to achieve a proper high level of strength in his finished paper product. This makes the final sheet product more expensive as the long fiber is generally more expensive than a short fiber. In essence, the separation of paper manufacturer from forms manufacturer, which is now common, requires that the paper manufacturer overdesign his final product for a variety of machines, instead of specifically designing the paper product for known machine conditions.

By combining the manufacturing, printing and finishing operations into a single on-line system a number of advantages are achieved. First, the paper can be made using ground wood and a lower long fiber to short fiber ratio as was developed supra. This is a cost and potentially a quality improvement in the final paper product. A second advantage which can be derived from a combination of manufacturing, printing and finishing is that waste or re-cycled paper hereinafter sometimes referred to as "broke" can be used in the manufacture of the paper since the quality of the paper is not of an over-designed high standard. Third and most importantly, several steps in the normal process of the manufacture of forms can be completely eliminated. Specifically, drying steps can be eliminated by using a non-aqueous, solvent-free coating system and in addition, the warehousing and shipping steps can be avoided, thus resulting in a more cost efficient product.

Additionally, by using appropriate coating methods, namely radiation curable coating compositions and methods, and by combining the necessary manufacturing and printing steps, spot printing and spot coating can be realized. Both of these represent a significant cost savings but nevertheless one which is not generally available when aqueous coatings are used or where the manufacture, printing and finishing of paper are performed as separate functions. An additional advantage of the use of radiation curable coating compositions and the combination of paper manufacturer, printer and finisher is that when the option of printing followed by coating is available significant cost advantages occur.

#### STATEMENT OF THE INVENTION

In one aspect of the invention, a process is provided for the production of a coating composition containing microcapsules having a hydrophilic core for use in the manufacture of pressure-sensitive carbonless transfer papers comprising the following steps. A hydrophilic emulsion component is prepared by dispersing at least one chromogenic material in a hydrophilic liquid, the chromogenic material being soluble in the hydrophilic liquid. A hydrophobic emulsion component is prepared by dispersing an emulsifier in a radiation curable hydrophobic liquid. A first wall-forming material and a second wall-forming material are added to the hydrophobic emulsion component, with mixing. The first and second wall-forming materials are soluble in the hydrophobic emulsion component, and the first wall-forming material is reactive with the second wall-forming material to form a polymeric capsule wall. The resultant polymeric capsule wall is substantially insoluble in the hydrophilic and the hydrophobic emulsion components. The hydrophobic emulsion component is mixed together with the hydrophilic emulsion component to form an emulsion containing droplets of the hydrophilic emulsion component dispersed in the hydrophobic emulsion component. Mixing is maintained for a period of time sufficient to allow the first and second wall-forming materials to react to form a dispersion of microcapsules in the hydrophobic emulsion component. The formed microcapsules have capsule walls substantially impermeable to the hydrophobic and the hydrophilic emulsion components.

In another aspect of the invention, pressure-sensitive carbonless transfer paper may be produced by applying the dispersion of the microcapsules prepared as above to a substrate, and curing the dispersion by subjecting the dispersion on the substrate to radiation for a period

of time sufficient to cure the radiation curable hydrophobic liquid, thereby producing a tack-free, resinous film on the substrate.

### DETAILED DESCRIPTION OF THE INVENTION

The coating composition of this invention is essentially a dispersion of microcapsules containing a chromogenic material or materials dissolved in a hydrophilic liquid in a radiation curable hydrophobic liquid as a continuous phase. The dispersion of microcapsules is prepared in situ in the radiation curable hydrophobic liquid by reaction of a first wall-forming material and a second wall-forming material both present in the radiation curable hydrophobic liquid. For purposes of this application, the term "chromogenic" shall be understood to refer to materials such as color precursors, color developers, and color formers.

The coating composition can contain additional materials which function as photoinitiators. Addition of these materials depends upon the particular method of curing the microcapsular coating. Filler materials can also be added to modify the properties of the cured film. The use of non-reactive solvents for the radiation curable liquid, which require heat to remove them during the drying or curing of the coated film, is avoided. However, minor amounts of nonreactive solvents can be tolerated without requiring a separate step for drying during any subsequent curing step. Although the product and process of this invention are useful in the manufacture of a variety of microencapsulated products, the preferred use of the process and product of this invention is in the production of a pressure-sensitive carbonless transfer sheets such as is described in commonly-assigned co-pending U.S. application Ser. No. 684,462, filed May 7, 1976.

In general, the hydrophilic liquids known in the art, as illustrated by those listed in U.S. Pat. No. 3,432,427 to Kan et al., can be used in the practice of this invention. Examples of the preferred hydrophilic liquids are water, glycerin, 1,4-butanediol, polyethylene glycol, 1,2-propylene glycol, 2,3-butylene glycol, polypropylene glycol, triethylene glycol, triethylene glycol monomethyl ether, diethylene glycol, ethylene diamine, triethylene diamine, diethylene triamine, triethylene tetraamine, tetraethylene pentamine, polyethylenimine and mixtures thereof.

In the preferred use of this invention to prepare pressure-sensitive transfer sheets, the most preferred hydrophilic liquid is a mixture of water and glycerin. The hydrophilic liquid also contains at least one chromogenic material dissolved therein. Besides being soluble in the hydrophilic liquid, the chromogenic materials should be essentially insoluble in the hydrophobic liquid and should not be substantially reactive to any appreciable degree with the other ingredients of the coating composition, such as the hydrophilic liquid, the radiation curable substance and the wall-forming materials. The chromogenic material can be selected from any color-forming pair in which one chromogenic material reacts with another chromogenic material in the presence of the hydrophilic liquid to form a color. Following are pairs in which the first mentioned chromogenic material is particularly useful in the practicing of this invention. A most preferred chromogenic material is sodium orthovanadate.

| Color Former Pairs                               | COLOR        |
|--------------------------------------------------|--------------|
| Ammonium ferric sulfate - Potassium ferrocyanide | Blue         |
| Ammonium ferric sulfate - Potassium thiocyanate  | Red brown    |
| Ammonium ferric sulfate - Salicyaldoxime         | Brown        |
| Ammonium ferric sulfate - Gallic acid            | Black        |
| Ammonium ferric sulfate - Tannic acid            | Black        |
| Ammonium ferric sulfate - Catechol               | Black        |
| Ammonium ferric sulfate - 8-Hydroxyquinoline     | Black        |
| Ferric oleate - Catechol                         | Violet-Black |
| Ferric oleate - Sodium diethyldithiocarbonate    | Black        |
| Sodium orthovanadate - 2-Ethylhexyl gallate      | Black        |
| Sodium orthovanadate - Gallic acid               | Black        |
| Ammonium metavanadate - Gallic acid              | Black        |
| Ammonium metavanadate - Tannic acid              | Black        |
| Ferric sulfate - 2,4-dinitro-1-naphthol          | Black        |
| Cupric sulfate - Dithioxamide                    | Black        |
| Cupric oleate - Dithioxamide                     | Black        |

15

The chromogenic materials are present in the hydrophilic liquid in an amount from about 0.2 to 10% based on the weight of the hydrophilic liquid. The most preferred range is from about 0.5 to about 4.0%.

The radiation curable liquids useful in the practice of this invention comprise the free radical polymerizable ethylenically unsaturated organic compounds. These compounds contain at least one terminal ethylenically unsaturated group per molecule. These compounds are hydrophobic liquids and function as a continuous hydrophobic phase during the in situ preparation of the microcapsules and as a dispersing medium for the microcapsules and other ingredients of the coating composition prior to the coating operation. They are non-reactive with the wall-forming materials and they are curable to a solid resin when exposed to ionizing or ultraviolet radiation. Thus the cured resin acts as a binder for the microcapsules to a substrate such as paper.

A group of useful radiation curable compounds are the polyfunctional ethylenically unsaturated organic compounds which have more than one (two or more) terminal ethylenic groups per molecule. Due to the polyfunctional nature of these compounds, they cure rapidly under the influence of radiation by polymerization, including cross-linking, to form a hard, dry, tack-free film.

Included in this group of radiation curable compounds are the polyesters of ethylenically unsaturated acids such as acrylic acid and methacrylic acids, and a polyhydric alcohol. Examples of some of these polyfunctional compounds are the polyacrylates or methacrylates of trimethylolpropane, pentaerythritol, dipentaerythritol, ethylene glycol, triethylene glycol, propylene glycol, glycerin, sorbitol, neopentylglycol and 1,6-hexanediol, hydroxy-terminated polyesters, hydroxy-terminated epoxy resins, and hydroxy-terminated polyurethanes and polyphenols such as bisphenol A.

Also included in this group are polyallyl and polyvinyl compounds such as diallyl phthalate and tetraallyloxyethane, and divinyl adipate, butane divinyl ether and divinylbenzene. Mixtures of these polyfunctional compounds and their oligomers and prepolymers may be used if desired.

Another group of radiation curable compounds which are useful are the monofunctional ethylenically unsaturated organic compounds which have one terminal ethylenic group per molecule. Examples of such monofunctional compounds are the  $C_2$  to  $C_{16}$  alcohol esters of acrylic and methacrylic acid, and styrene, substituted styrenes, vinyl acetate, vinyl ethers and allyl phenols. In general, these compounds are liquid and have a lower viscosity than the polyfunctional ethyleni-

cally unsaturated compound and thus may be used to reduce the viscosity of the coating composition to facilitate migration of the wall-forming materials during preparation of the microcapsules. These compounds are radiation curable and react with the ethylenically unsaturated polyfunctional organic compounds during radiation curing to give a dry flexible film. Compounds having only one terminal ethylenic group may be used alone as the radiation curable hydrophobic liquid. However, the resultant radiation cured film may be rather soft and pliable and hence less preferred commercially than other ethylenically unsaturated compounds.

The preferred radiation curable hydrophobic liquid is a mixture containing one or more monofunctional compounds and one or more polyfunctional compounds. The monofunctional compounds due to their generally lower viscosity, tend to more easily disperse the hydrophilic liquid into droplets of the desired size. The polyfunctional compounds tend to cure more rapidly and due to cross-linking give a harder tougher resin film. This is particularly so when compounds of higher molecular weight, such as the oligimers and prepolymers of the polyfunctional compounds, are used. In a preferred process of this invention, the lower viscosity monofunctional compounds are used as the dispersing media for the preparation of the microcapsules and the higher viscosity, faster curing polyfunctional compounds, particularly the oligimers and prepolymers of these compounds, are added after the microcapsules are formed and prior to coating on a substrate.

The radiation curable hydrophobic liquid can be present in the microcapsular coating composition in an amount of from about 25 to about 75% by weight of the composition. The preferred range is from about 35 to about 65% and the most preferred range is from about 40 to about 55%.

The radiation curable hydrophobic liquid acts as the continuous or external phase in the in situ formation of the microcapsules. The first and second wall-forming materials are compatible with the radiation curable hydrophobic liquid. These first and second wall-forming materials are reactive with each other to form a polymer insoluble in hydrophilic and hydrophobic liquids. The first wall-forming material can be selected from the group consisting of polyols, epoxy compounds, polythiols, polyamines, acid anhydrides, and polycarboxylic acids, and mixtures thereof. The polyols include, for example, resorcinol, 1,3-naphthalenediol, bisphenol A, 1,3-propylene glycol, 1,5-pentanediol and the like. The epoxy compounds are, for example, diglycidyl ether, glycerin triglycidyl ether and diglycidyl ether of bisphenol A. Examples of polythiols, are thioglycol and thioglycol condensates. Polyamines include, for example, p-phenyleneamine, and phthalamide and the like. Examples of acid anhydrides include maleic anhydride and succinic anhydride. Examples of polycarboxylic acids are malonic acid, succinic acid and tetraphthalic acid. The preferred first wall-forming material are the polyols. The second wall-forming material is a polyisocyanate and may include (a) diisocyanates, such as m-phenylmethane-4,4'-diisocyanate; (b) triisocyanates, such as toluene-2,4,6-triisocyanate; (c) tetraisocyanates, such as 2,2',5,5'-tetraisocyanate; (d) isocyanate prepolymers such as Desmodur E-21 (an aromatic polyisocyanate prepolymer produced and sold by Mobay Chem. Co.), Mondur CB-75 (75% of a high molecular weight adduct of toluene isocyanate and 25% of ethyl acetate produced and sold by Mobay

Chem. Co.), and Desmodur N-100 (a biuret containing aliphatic isocyanate produced and sold by Mobay Chem. Co.). The radiation curable hydrophobic liquid may also contain a catalyst to promote the reaction of the first and second wall-forming materials. Such catalysts include amines, organo-metallic compounds and various organic acid salts of metals.

A photoinitiator is added to the coating composition if the composition is to be cured by ultraviolet radiation. A wide variety of photoinitiators are available which serve well in the system described in this invention. The preferred photoinitiators are the benzoin alkyl ethers, such as Vicure 30 (a mixture of alkylbenzoin ethers manufactured and sold by Stauffer Chemical Co., Westport, Conn.), benzoin butyl ether (Vicure 10, Stauffer), benzoin methyl ether, and  $\alpha,\alpha$ -diethoxyacetophenone. Other photoinitiators which can be used are benzophenone, 4,4'-bis(dimethylamino)benzophenone, ferrocene, xanthone, thioxanthane,  $\alpha,\alpha$ -azobisisobutylnitrile, decabromodiphenyl oxide, pentabromomonochlorocyclohexane, pentachlorobenzene, polychlorinated biphenyls such as the Arochlor 1220 series (manufactured and sold by Monsanto Chemical Co., St Louis, Mo.), benzoin ethyl ether, 2-ethyl anthroquinone, 1-(chloroethyl) naphthalene, desyl chloride, chlorodic anhydride, naphthalene sulfonyl chloride and 2-bromoethyl ethyl ether. The amount of photoinitiator added can be from about 0.2 to about 10% by weight of the coating composition, with a preferred range from about 1 to about 8% by weight.

Photoinitiation synergists can also be added to the ultraviolet curable coating compositions. Photoinitiation synergists serve to enhance the initiation efficiency of the photoinitiators. The preferred synergists are the chain transfer agents, such as the tertiary alcoholamines and substituted morpholines, triethanolamine, N-methyldiethanolamine, N,N-dimethyllethanolamine and N-methylmorpholine. The amount of photoinitiation synergist added can be from about 0.2 to about 10% by weight of the coating composition, with a preferred range of from about 3 to about 8% by weight.

In the preparation of the microcapsules, a hydrophobic emulsion component is prepared by dissolving or dispersing an emulsifier in the radiation curable hydrophobic liquid. A hydrophilic emulsion component is prepared by dissolving the chromogenic material in water or other aqueous media. Preparation of each of these emulsion components is easily accomplished by stirring together at room temperature the materials of each component. The Brookfield viscosity of the hydrophobic emulsion component can be from about 0.5 cps. to about 1000 cps. The preferred viscosity is about 1 cps. to about 500 cps. and the most preferred viscosity is from about 1 cps. to about 50 cps.

The hydrophobic and hydrophilic emulsion components, which are two immiscible liquids, are mixed together with high agitation to form droplets of the hydrophilic emulsion component in the hydrophobic emulsion component. The hydrophilic emulsion component contains a hydrophilic carrier liquid and dissolved therein the chromogenic material. The hydrophobic emulsion component contains radiation curable hydrophobic liquid and an emulsifying agent. At this point the hydrophobic emulsion component may or may not contain the first and second wall-forming material. These wall-forming materials can be added to the hydrophobic emulsion component prior to emulsification or, alternatively, they may be added to the hydro-

phobic emulsion component (continuous phase) after the emulsification step. To facilitate mixing, both the first and the second wall-forming material may be dissolved or dispersed in additional radiation curable hydrophobic liquid prior to this addition. In any event, both the first and second wall-forming material must be soluble in the radiation curable hydrophobic liquid. The term "soluble" as used herein is intended to describe wall-forming materials which are only partially soluble in and give hazy solutions in the radiation curable hydrophobic liquid as well as those which are completely soluble in the radiation curable hydrophobic liquid.

After emulsification, the emulsion is stirred for a period of about 3 hours to about 16 hours at a temperature of about 0° to about 60° C., preferably room temperature to about 40° C., to allow the first and second wall-forming materials to react and form a dispersion of microcapsules having capsule walls which are substantially impermeable to both the hydrophilic and hydrophobic emulsion components used to form the microcapsules. The microcapsules should be from about 0.1 micron to about 50 microns in diameter. A preferred range is from about 5 to 15 microns.

A catalyst to promote the reaction of the first and second wall-forming materials may be added if desired to the hydrophobic emulsion component prior to emulsification. Such catalysts are known from U.S. Pat. No. 3,796,669 mentioned supra and include amines, organometallic compounds, various organic salts of metals, tertiary phosphine, alkaline metal compounds, and radical forming agents. A preferred catalyst is dibutyl tin laurate.

In a preferred embodiment of the process of this invention, the radiation curable hydrophobic liquid is divided into two portions and the first portion is present in the hydrophobic emulsion component prior to the emulsification step. A second portion of the radiation curable hydrophobic liquid containing, in particular, faster curing polyfunctional oligimers and prepolymers may be added after the microcapsules are formed. At this point, other materials such as the photoinitiation synergists may be added to give a coatable composition. Stilt material may be added, if desired, to prevent premature rupture of the microcapsules.

The microcapsular coating composition of this invention can be applied to a substrate, such as paper or a plastic film by any of the common paper coating processes such as roll, air knife, or blade coating, or by any of the common printing processes, such as offset, gravure, or flexographic printing. The rheological properties, particularly the viscosity, of the coating composition, can be adjusted for each type of application by proper selection of the type, molecular weight and relative amounts of the liquid radiation curable compounds.

These coating compositions can be cured by any free radical initiated chain propagated addition polymerization reaction of the terminal ethylenic groups of the radiation curable compounds. These free radicals can be produced by several different chemical processes including the thermal or ultraviolet induced degradation of a molecular species and any form of ionizing radiation such as alpha-particles, beta-rays (high-energy electrons), gamma-rays, X-rays and neutrons.

The preferred curing process is by exposure of the coating composition to ultraviolet radiation having a wavelength of about 2000 Å to about 4000 Å. For curing to occur the composition must contain suitable ul-

traviolet absorbing photoinitiators which will produce polymerization initiating free radicals upon exposure to the radiation source. A typical ultraviolet source suitable for this type of curing process is a Hanovia 200 watt medium pressure mercury lamp. Curing efficiencies of the coating composition are dependent on such parameters as the nature of the radiation curable substance, atmosphere in contact with the coating, quantum efficiency of the radiation absorbed, thickness of coating and inhibitory effects of the various materials in the composition.

In the ionizing radiation induced curing of these coating compositions a specific radiation absorbing material (photoinitiator) is not necessary. Exposure of the coating composition to a source of high energy electrons results in spontaneous curing of the composition to a tough, tack-free coating. Any of a number of commercially available high energy electron beam or linear cathode type high energy electron sources are suitable for curing these compositions. Parameters such as the atmospheric environment and inhibitory effects of the various materials in the composition play an important role in the determination of the curing efficiency of these compositions.

The following examples further illustrate but do not limit the invention:

#### EXAMPLE 1

In 30 parts of distilled water was dissolved 2.1 parts of vanadium pentoxide, 3.9 parts of sodium hydroxide, 60 parts of glycerin and 40 parts of sodium bromide (Liquid A). The vanadium pentoxide and sodium hydroxide combine to form the chromogenic material, sodium orthovanadate. The glycerin and sodium bromide are added to prevent loss of the aqueous phase. To 150 parts of 2-ethylhexyl acrylate (radiation curable compound) was added 1.5 parts of a mixture of glycerol stearate and polyoxyethylene stearate (an emulsifying agent sold under the trade name Arlacel 165 by I.C.I. United States, Inc., Wilmington, Del.) and stirred at room temperature. A cloudy mixture (Liquid B) was obtained. The Brookfield viscosity of Liquid B at 25° C was 12 centipoise.

A solution of 22.5 parts of Mondur CB-60 (a 61% solution in a mixture of xylene and 2-ethoxyethyl acetate of a toluene diisocyanate-based adduct made and sold by Mobay Chemical Co., Pittsburgh Pa.) and 2.4 parts of dipropylene glycol (polyol) were dissolved in 75 parts of 2-ethylhexyl acrylate at room temperature to give a clear solution (Liquid C).

Liquid B was placed in a Waring Blender. Liquid A was slowly added to Liquid B in the Waring blender while running at high speed. The emulsification was continued for 2 minutes. Liquid C was then added slowly at high speed and mixed for 3 more minutes. The resultant emulsion was then transferred to a 3-neck glass reactor which was equipped with a condenser and a mechanical stirrer. The emulsion was stirred overnight (about 16 hours) at 40° C to yield a dispersion of microcapsules.

To 60 parts of this microcapsular dispersion was added 8 parts of Ucar Actomer X-80 (a polyfunctional acrylate oligomer made and sold by Union Carbide Corporation, New York, N.Y.), 10 parts of Keestar 339 (an antimudge agent made and sold by A. E. Staley Mfg. Co., Decatur, Illinois), and 2.4 parts of Vicure 30 and the mixture (coating composition) was applied on a sheet of polyvinyl alcohol basecoated paper with a #19

Mayer bar. The sheet was exposed to ultraviolet light, light which was generated by the ultraviolet QC 1202 AN Processor (manufactured and sold by Radiation Polymer Co., a division of PPG Industries, Pittsburgh, Pa.).

Another coating composition was made as mentioned above except that the Vicure 30 was omitted. This coating composition was then coated with a #22 Mayer bar to a polyvinyl alcohol basecoated paper and cured by a linear cathode electron beam processor at Radiation Polymer Co. which was operated at 5 megarads, 230 KV, and a speed of 50 ft. per minute using a nitrogen blanket.

The ultraviolet light cured and electron beam cured transfer sheets each performed satisfactorily as transfer sheets of a carbonless paper system using a 2-ethylhexyl gallate coated record sheet.

#### EXAMPLE 2

In 30 parts of distilled water, 2.1 parts of vanadium pentoxide, 3.9 parts of sodium hydroxide, 60 parts of glycerin and 40 parts of sodium bromide were dissolved (Liquid A). To 175 parts of 2-ethylhexyl acrylate was added 2 parts of Arlacet 165, 2.4 parts of dipropylene glycol (polyol) and 22.5 parts of Mondur CB-60 (polyisocyanate) and stirred at room temperature. A cloudy mixture (Liquid B) was obtained.

Liquid A was then emulsified into Liquid B for 4 minutes in a Waring blender at high speed. The emulsion was then transferred into a glass reactor to cure overnight (about 16 hours) at 40°-44° C.

To 60 parts of this microcapsular dispersion was added 8 parts of Ucar Actomer X-80, 10 parts of Kee-star 339 and 2.4 parts of Vicure 30 and the mixture was applied on a sheet of polyvinyl alcohol basecoated paper with a #19 Mayer bar. The sheet was exposed to the ultraviolet QC 1202 AN Processor.

Another coating composition was made as mentioned above except no Vicure 30 in the mixture. This coating composition was then coated with a #22 Mayer bar to a polyvinyl alcohol basecoated paper and cured by a linear cathode electron beam processor at Radiation Polymer Co., which was operated at 5 megarads, 230 KV and a speed of 50 ft. per minute using a nitrogen blanket.

The ultraviolet light cured and electron beam cured transfer sheets each performed satisfactorily as a part of a carbonless paper system using a 2-ethylhexyl gallate coated record sheet.

What is claimed is:

1. A process for producing a liquid substantially solvent-free coating composition for use in the manufacture of pressure-sensitive carbonless transfer papers, said liquid coating composition being characterized by being radiation curable by polymerization to a dry, solid, tack-free resin substantially without the removal of solvents and other liquids and being further characterized by containing microcapsules having a hydrophilic core material, comprising the steps of:

(a) preparing a liquid hydrophilic emulsion component by dispersing at least one chromogenic material in a hydrophilic liquid, said chromogenic material being soluble in said hydrophilic liquid;

(b) preparing a liquid hydrophobic emulsion component by dispersing an emulsifier in a radiation curable hydrophobic liquid;

(c) adding to said liquid hydrophobic emulsion component, with mixing, a first wall-forming material

and second wall-forming material, said first and second wall-forming materials being soluble in said liquid hydrophobic emulsion component, said first wall-forming material being reactive with said second wall-forming material to form a polymeric capsule wall, said polymeric capsule wall being substantially insoluble in said liquid hydrophilic and said liquid hydrophobic emulsion components;

10 (d) mixing said liquid hydrophobic emulsion component with said liquid hydrophilic emulsion component to form an emulsion containing droplets of said liquid hydrophilic emulsion component dispersed in said liquid hydrophobic emulsion component; and

15 (e) maintaining said mixing for a period of time sufficient to allow said first and second wall-forming materials to react to form a dispersion of microcapsules in said liquid hydrophobic emulsion component, said microcapsules having capsule walls substantially impermeable to said liquid hydrophobic and said liquid hydrophilic emulsion components.

20 2. The process of claim 1 wherein said first and second wall-forming materials are added to said liquid hydrophobic emulsion component after said mixing of said liquid hydrophobic emulsion component with said liquid hydrophilic emulsion component.

25 3. The process of claim 1 wherein said radiation curable hydrophobic liquid comprises at least one ethylenically unsaturated organic compound having at least one terminal ethylenic group per molecule.

30 4. The process of claim 1 wherein said first wall-forming material is a member of the group consisting of polyols, polythiols, polyamines, acid anhydrides, polycarboxylic acids, and epoxy compounds and said second wall-forming material is a polyisocyanate.

35 5. The process of claim 4 wherein said first wall-forming material is a polyol.

40 6. The process of claim 1 wherein said chromogenic material is a color former selected from the group consisting of ammonium ferric sulfate, ferric oleate, sodium orthovanadate, ammonium metavanadate, ferric sulfate, cupric sulfate, cupric oleate and mixtures thereof.

45 7. The process of claim 1 wherein a catalyst capable of promoting the reaction of said first wall-forming material with said second wall-forming material is added to said emulsion prior to the reaction of said first wall-forming material with said second wall-forming material.

50 8. A process for producing a liquid substantially solvent-free coating composition for use in the manufacture of pressure-sensitive carbonless transfer papers, said liquid coating composition being characterized by being radiation curable by polymerization to a dry, solid, tack-free resin substantially without the removal of solvents and other liquids and being further characterized by containing microcapsules having a hydrophilic core material, comprising the steps of:

(a) preparing a liquid hydrophilic emulsion component by dispersing at least one chromogenic material in a hydrophilic liquid, said chromogenic material being soluble in said hydrophilic liquid;

(b) preparing a liquid hydrophobic emulsion component by dispersing an emulsifier in a first portion of a radiation curable hydrophobic liquid, said liquid hydrophobic emulsion component having a viscosity from about 1 centipoise to about 500 centipoise, said radiation curable hydrophobic liquid comprising at least one ethylenically unsaturated organic

- compound having at least one terminal ethylenic group per molecule;
- (c) adding to said liquid hydrophobic emulsion component, with mixing, at least one polyol and at least one polyisocyanate, said polyol and said polyisocyanate being soluble in said liquid hydrophobic emulsion component, said polyol being reactive with said polyisocyanate to form a polymeric capsule wall, said polymeric capsule wall being substantially insoluble in said liquid hydrophilic and said liquid hydrophobic emulsion components; 5
- (d) mixing said liquid hydrophobic emulsion component with said liquid hydrophilic emulsion component to form an emulsion containing droplets of said liquid hydrophilic emulsion component dispersed in said liquid hydrophobic emulsion component; 15
- (e) maintaining said mixing for a period of time sufficient to allow said polyol and said polyisocyanate to react to form a dispersion of microcapsules in 20 said liquid hydrophobic emulsion component, said microcapsules having capsule walls substantially impermeable to said liquid hydrophobic and said liquid hydrophilic emulsion components; and
- (f) adding to said dispersion of said microcapsules in 25 said liquid hydrophobic emulsion component a second portion of a radiation curable hydrophobic liquid, said second portion including at least one ethylenically unsaturated organic compound having more than one terminal ethylenic group per 30 molecule.

9. The process of claim 8 wherein a photoinitiator is added to said dispersion of microcapsules.

10. A process for producing a liquid substantially solvent-free coating composition for use in the manufacture of pressure-sensitive carbonless transfer papers, said liquid coating composition being characterized by being radiation curable by polymerization to a dry solid, tack-free resin substantially without the removal of solvents and other liquids and being further characterized by containing microcapsules having a hydrophilic core material, comprising the steps of: 35

- (a) preparing a liquid hydrophilic emulsion component by dispersing at least one chromogenic material in a hydrophilic liquid, said chromogenic material being soluble in said hydrophilic liquid; 45
- (b) preparing a liquid hydrophobic emulsion component by dispersing an emulsifier in a first portion of a radiation curable hydrophobic liquid, said liquid hydrophobic emulsion component having a viscosity from about 1 centipoise to about 500 centipoise, said radiation curable hydrophobic liquid comprising at least one ethylenically unsaturated organic compound having at least one terminal ethylenic group per molecule; 50
- (c) mixing said liquid hydrophobic emulsion component with said liquid hydrophilic emulsion component to form an emulsion containing droplets of said liquid hydrophilic emulsion component dispersed in said liquid hydrophobic emulsion component; 60
- (d) adding at least one polyol and at least one polyisocyanate to said liquid hydrophobic emulsion component with further mixing, said polyol and said polyisocyanate being soluble in said liquid hydrophobic emulsion component, said polyol being reactive with said polyisocyanate to form a polymeric capsule wall, said polymeric capsule wall 65

being substantially insoluble in said liquid hydrophilic and said liquid hydrophobic emulsion components;

- (e) maintaining said mixing for a period of time sufficient to allow said polyol and said polyisocyanate to react to form a dispersion of microcapsules in said liquid hydrophobic emulsion component, said microcapsules having capsule walls being substantially impermeable to said liquid hydrophobic and said liquid hydrophilic emulsion components; and
- (f) adding to said dispersion of said microcapsules in said liquid hydrophobic emulsion component a second portion of a radiation curable hydrophobic liquid, said second portion including at least one ethylenically unsaturated organic compound having more than one terminal ethylenic group per molecule.

11. The process of claim 10 wherein a photoinitiator is added to said dispersion of microcapsules.

12. A process for producing a pressure-sensitive carbonless transfer paper comprising the steps of:

- (a) preparing a liquid hydrophilic emulsion component by dispersing at least one chromogenic material in a hydrophilic liquid, said chromogenic material being soluble in said hydrophilic liquid;
- (b) preparing a liquid hydrophobic emulsion component by dispersing an emulsifier in a radiation curable hydrophobic liquid;
- (c) adding to said liquid hydrophobic emulsion component, with mixing, a first wall-forming material and second wall-forming material, said first and second wall-forming materials being soluble in said liquid hydrophobic emulsion component, said first wall-forming material being reactive with said second wall-forming material to form a polymeric capsule wall, said polymeric capsule wall being substantially insoluble in said liquid hydrophilic and said liquid hydrophobic emulsion components;
- (d) mixing said liquid hydrophobic emulsion component with said liquid hydrophilic emulsion component to form an emulsion containing droplets of said liquid hydrophilic emulsion component dispersed in said liquid hydrophobic emulsion component;
- (e) maintaining said mixing for a period of time sufficient to allow said first and second wall-forming materials to react to form a dispersion of microcapsules in said liquid hydrophobic emulsion component, said microcapsules having capsule walls substantially impermeable to said liquid hydrophobic and said liquid hydrophilic emulsion components;
- (f) applying said dispersion of said microcapsules to a substrate; and
- (g) curing said dispersion of said microcapsules by subjecting said dispersion of said microcapsules on said substrate to radiation for a period of time sufficient to cure said dispersion of said microcapsules by polymerization of said radiation curable hydrophobic liquid, thereby producing a dry, solid, tack-free resinous film on said substrate substantially without the removal of solvents or other liquids.

13. The process of claim 12 wherein said first and second wall-forming materials are added to said liquid hydrophobic emulsion component after said mixing of said liquid hydrophobic emulsion component with said liquid hydrophilic emulsion component.

14. The process of claim 12 wherein said radiation curable hydrophobic liquid comprised at least one eth-

ylenically unsaturated organic compound having at least one terminal ethylenic group per molecule.

15. The process of claim 12 wherein said first wall-forming material is a polyol and said second wall-forming material is a polyisocyanate.

16. The process of claim 12 wherein said chromogenic material is selected from the group consisting of ammonium ferric sulfate, ferric oleate, sodium orthovanadate, ammonium metavanadate, ferric sulfate, cupric sulfate, cupric oleate and mixtures thereof.

17. The process of claim 12 wherein a catalyst capable of promoting the reaction of said first wall-forming material with said second wall-forming is added to said emulsion prior to the reaction of said first wall-forming material with said second wall-forming material.

18. A process for producing a pressure-sensitive carbonless transfer paper comprising the steps of:

- (a) preparing a liquid hydrophilic emulsion component by dispersing at least one chromogenic material in a hydrophilic liquid, said chromogenic material being soluble in said hydrophilic liquid;
- (b) preparing a liquid hydrophobic emulsion component by dispersing an emulsifier in a radiation curable hydrophobic liquid, said liquid hydrophobic emulsion component having a viscosity from about 1 centipoise to about 500 centipoise, said radiation curable hydrophobic liquid comprising at least one ethylenically unsaturated organic compound having at least one terminal ethylenic group per molecule;
- (c) adding to said liquid hydrophobic emulsion component, with mixing, at least one polyol and at least one polyisocyanate, said polyol and said polyisocyanate being soluble in said liquid hydrophobic emulsion component, said polyol being reactive with said polyisocyanate to form a polymeric capsule wall, said polymeric capsule wall being substantially insoluble in said liquid hydrophilic and said liquid hydrophobic emulsion components;
- (d) mixing said liquid hydrophobic emulsion component with said liquid hydrophilic emulsion component to form an emulsion containing droplets of said liquid hydrophilic emulsion component dispersed in said liquid hydrophobic emulsion component;
- (e) maintaining said mixing for a period of time sufficient to allow said polyol and said polyisocyanate to react to form a dispersion of microcapsules in said liquid hydrophobic emulsion component, said microcapsules having capsule walls substantially impermeable to said liquid hydrophobic and said liquid hydrophilic emulsion components;
- (f) applying said dispersion of said microcapsules to a paper substrate; and
- (g) curing said dispersion of said microcapsules by subjecting said dispersion of said microcapsules on said paper substrate to radiation for a period of time sufficient to cure said dispersion of said microcapsules by polymerization of said radiation curable hydrophobic liquid, thereby producing a dry, solid, tack-free resinous film on said paper substrate substantially without the removal of solvents or other liquids.

19. The process of claim 18 wherein said radiation curable hydrophobic liquid comprises a mixture of ethylenically unsaturated organic compounds, a portion of said compounds having one terminal ethylenic group per molecule and another portion of said compounds

having more than one terminal ethylenic group per molecule.

20. The process of claim 18 wherein a photoinitiator is added to said dispersion of microcapsules and said radiation is ultraviolet light.

21. A process for producing a pressure-sensitive carbonless transfer paper comprising the steps of:

- (a) preparing a liquid hydrophilic emulsion component by dispersing at least one chromogenic material in a hydrophilic liquid, said chromogenic material being soluble in said hydrophilic liquid;
- (b) preparing a liquid hydrophobic emulsion component by dispersing an emulsifier in a radiation curable hydrophobic liquid, said liquid hydrophobic emulsion component having a viscosity from about 1 centipoise to about 500 centipoise, said radiation curable hydrophobic liquid comprising at least one ethylenically unsaturated organic compound having at least one terminal ethylenic group per molecule;
- (c) mixing said liquid hydrophobic emulsion component with said liquid hydrophilic emulsion component to form an emulsion containing droplets of said liquid hydrophilic emulsion component dispersed in said liquid hydrophobic emulsion component;
- (d) adding at least one polyol and at least one polyisocyanate to said liquid hydrophobic emulsion component with further mixing, said polyol and said polyisocyanate being soluble in said hydrophobic liquid, said polyol being reactive with said polyisocyanate to form a polymeric capsule wall, said polymeric capsule wall being substantially insoluble in said liquid hydrophilic and said liquid hydrophobic emulsion components;
- (e) maintaining said mixing for a period of time sufficient to allow said polyol and said isocyanate to react to form a dispersion of microcapsules in said liquid hydrophobic emulsion component, said microcapsules having capsule walls substantially impermeable to said liquid hydrophobic and said liquid hydrophilic emulsion components;
- (f) applying said dispersion of said microcapsules to a paper substrate; and
- (g) curing said dispersion of said microcapsules by subjecting said dispersion of said microcapsules on said paper substrate to radiation for a period of time sufficient to cure said dispersion of said microcapsules, by polymerization of said radiation curable hydrophobic liquid, thereby producing a dry, solid, tack-free resinous film on said paper substrate substantially without the removal of solvents or other liquids.

22. The process of claim 21 wherein said radiation curable hydrophobic liquid comprises a mixture of ethylenically unsaturated organic compounds, a portion of said compounds having one terminal ethylenic group per molecule and another portion of said compounds having more than one terminal ethylenic group per molecule.

23. The process of claim 21 wherein a photoinitiator is added to said dispersion of microcapsules and said radiation is ultraviolet light.

24. The pressure-sensitive carbonless transfer paper produced by the process of claim 18.

25. The pressure-sensitive carbonless transfer paper produced by the process of claim 21.

\* \* \* \* \*